

# UNITED STATES PATENT OFFICE.

PAUL MORITZ KRAIS, OF ILKLEY, ENGLAND.

## SCHREINER FINISH OF TEXTILE FABRICS.

No. 922,295.

Specification of Letters Patent. Patented May 18, 1909.

Application filed December 16, 1903. Serial No. 185,438.

*To all whom it may concern:*

Be it known that I, PAUL MORITZ KRAIS, a subject of the Emperor of Germany, residing at Ilkley, in the county of York, in the 5 Kingdom of England (whose post-office address is 5 Easby Drive, Ilkley, aforesaid), have invented certain new and useful Improvements in Schreiner Finish of Textile Fabrics, for which application has been made 10 in Great Britain, No. 25,463, dated November 21, 1903.

Certain classes of piece goods have for many years been passed between rollers engraved with fine parallel lines in order to give 15 them a silk-like gloss or lustre, which is commonly known as "Schreiner finish." The gloss produced by such mechanical means is, however, fugitive, being more or less lost when the goods are exposed to a moist atmosphere, or to rain, or to the tailor's iron. For 20 many years past efforts have been made to render such mechanical finishes permanent, and many processes have been tried, but up to the present time only a very partial success has been obtained. Thoroughly 25 impregnating the materials with varnish or various forms of altered cellulose has been tried, whereby the fabric has been made waterproof. If this be done before schreining, a stiff, hard material is the result, 30 while if it be done after schreining the effect of the latter is to a considerable extent lost and the color of the material is also changed.

35 My invention is designed to leave the material almost entirely unaltered in texture and appearance, but yet to render the schreining permanent, and it consists essentially in treating the surface of the fabric after schreining with a fluid solution of 40 soluble nitro-cellulose in one of the usual solvents, preferably amyl acetate. In place of this solution I may, however, use other cellulose compounds which are soluble in 45 volatile organic solvents, such as acetate of cellulose or other ethers of cellulose or hydro-cellulose, or mixtures of the compounds named.

50 The solution is applied by spraying the schreined surface, but it is essential that the goods should not be substantially stiffened or their appearance materially altered. The solution is preferably applied twice in succession, the solvent being evaporated 55 after each application, but the spraying

should be such as not to form a skin over the fabric or render it waterproof. It should be in fact just sufficient to impregnate each individual fiber of the schreined surface of the cloth, and thus mechanically fix the produced luster. The result is that moisture will, though it may cause the fibers to swell, not separate them from the position in which they have been laid by the schreining, while at the same time the appearance of the 60 fabric is unaltered. I obtain the best and most perfect results with mercerized cotton pieces which have been dyed anilin black, and in order to preserve the full depth of the black I may tint the solution with a suitable 65 dyestuff soluble in the solvent used.

70 As an illustration, in carrying out my operation I spray a 5% solution diluted with its own volume of 96% amyacetate on the piece previously schreined and then evaporate and repeat the operation if necessary. I find the best result is obtained when the 75 respective weights of the cellulose substances remaining in the piece after evaporation and the piece itself are from 0.2% to 5% of the 80 cellulose compound to 100 of the piece.

Having thus described my invention, what I claim is:

1. The process of producing a permanent Schreiner finish on textile materials, which 85 consists in passing the material between rollers engraved with fine parallel lines and then treating the goods with an amyacetate solution of cellulose, the solution being of such strength or dilution that it does not sensibly 90 stiffen or waterproof the material as a whole while practically waterproofing the fibers of the schreined surface thereof.

2. The process of producing a permanent Schreiner finish on textile materials, which 95 consists in passing the material between rollers engraved with fine parallel lines; and then treating the surface of the goods with cellulose dissolved in a volatile organic solvent, the solution being of such strength or 100 dilution that it does not sensibly stiffen or waterproof the material as a whole while practically waterproofing the fibers of the schreined surface thereof.

3. The process of producing a permanent 105 Schreiner finish on textile materials, which consists in passing the material between rollers engraved with fine parallel lines; then repeatedly spraying the goods thus treated with a solution of cellulose dissolved in a 110

volatile organic solvent, the solution being extremely thin; and drying the material between each spraying, whereby the goods are not sensibly stiffened or waterproofed as a whole while practically the fibers of the schreinered surface are waterproofed.

4. The process herein described of finishing textile material, which consists in passing the material between engraved rollers; then 10 treating the material with a solution of nitro-cellulose in amyl-acetate; and finally evapo-

rating the solvent and thereby fixing or rendering permanent the finish produced by the rollers without waterproofing the material itself.

In witness whereof, I have hereunto signed my name this 2nd day of December 1903, in the presence of two subscribing witnesses.

PAUL MORITZ KRAIS.

Witnesses:

H. O. WADE,  
BERTRAM HOWE.